

Jan. 12, 1965

G. F. KOTRBATY

3,164,898

METHOD OF PRODUCING EXTRUDED SHAPES

Filed Aug. 9, 1960

2 Sheets-Sheet 1



**FIG. 2.**



**FIG. 5.**



**FIG. 4.**



**FIG. 3.**



**FIG. 7.**



BY

*Guy F. Kotrbaty*

ATTORNEY

INVENTOR

GUY F. KOTRBATY.

Jan. 12, 1965

G. F. KOTRBATY

3,164,898

METHOD OF PRODUCING EXTRUDED SHAPES

Filed Aug. 9, 1960

2 Sheets-Sheet 2

FIG. 8.



INVENTOR  
GUY F. KOTRBATY

BY *Guy F. Kotrbaty*  
ATTORNEY

1

3,164,898

**METHOD OF PRODUCING EXTRUDED SHAPES**  
Guy F. Kotrbaty, 56 Pondfield Road W.,  
Bronxville, N.Y.Filed Aug. 9, 1960, Ser. No. 48,438  
22 Claims. (Cl. 29—553)

This invention relates to an improved method of producing extruded shapes from metals and metal alloys, and more particularly to a novel method of producing finished extrusions of larger dimensions than the circumscribed diameter of the press die from which they are extruded.

In the currently employed method of producing extruded metallic shapes, such as aluminum, brass, copper, and magnesium base alloys, the maximum length, width and depth of the extrusion is limited essentially by three factors, namely, the effective pressure behind the ingots or billets, the weight and size of the ingot or billet and the circumscribed circle of the orifice of the die. In light of these limitations the preponderate number of extrusion presses in use are limited to a 12 in. container or less, while presses having an 8 in. or smaller die orifice account for approximately 95% of the extrusion presses in this country. The principal and compelling reason for this size limitation is the tremendous cost of extrusion presses that can extrude larger shapes. Extrusion presses having a container diameter of up to 24 in. have been built and operated by certain of the large aluminum producing companies. The cost of such installations ranges up to 20 million dollars and their installation and production costs are so high that they are feasible only for large runs or for important defense items. Major factors entering into such costs are the great expense of the precision dies employed and the relatively prolonged set-up and down-time involved in the production schedules. Furthermore, a limiting factor in the use of such larger presses is that the larger the circumscribed diameter die orifice of the press the more it is limited in producing shapes having thin wall sections. Hence the wider the section or shape required, the thicker the wall section must be, making it unduly heavy and costly, and uneconomical for most uses. In view of these factors, the vast majority of operators in the industry cannot assume the capital investment required for such large units, and hence they are presently excluded from the field of large circumscribed circle diameter extruded shapes, which field is now substantially preempted by the operators of ultra high pressure extruders.

With the rapidly increasing use of aluminum and its alloys in the many fields of construction, there is an increased demand for shapes of greater width and/or depth with thin wall sections than those heretofore produced by the extant relatively low pressure extruders. While larger shapes may be produced by fabrication from smaller extruded components, this not only involves additional cost incident to machining and joining the components, but the composite structural units thus produced do not achieve the performance and the many other advantages inherent in an integral extruded shape counterpart.

A major objective of the invention is to surmount the size limitation of an extruded metallic shape now imposed by current orthodox methods of production.

Another salient objective of the invention is to greatly expand the productive potential of presently installed metal extruders by deriving therefrom extruded shapes of a circumscribed circle diameter greater than that heretofore produced in such extruders.

Another objective of the invention is to materially increase the size of extruded metallic shapes utilizing currently installed extruders, by novel integration of the extruders with readily available accessory equipment.

Yet another objective of the invention is to produce

2

an extruded metal shape of novel design and configuration having masses or banks of metal amenable to post treatment to extend a selected dimension of the extruded shape.

Still another objective of the invention is to produce an extruded metal shape of novel design and configuration, efficiently utilizing the circular die area, which shape embodies web portions of selected cross-section, and ribs or banks of metal of greater cross-section, which ribs are amenable to post treatment to extend a selected dimension of the shape.

Another objective of the invention is to devise an improved process for producing extruded metallic shapes in which the ratio of the circumscribing diameter of the shape to the circumscribed diameter of the die orifice is at least 2 to 1.

A still further objective of the invention is to devise an improved method of producing extruded metallic shapes by a novel integration of preliminary extrusion, and subsequent selective cross-section reduction of portions of the shape.

With these and other equally important objectives in view, the invention comprehends the concept of extruding an intermediate shape comprised of portions of the desired ultimate cross-section and one or more integral portions of relatively greater cross section, which latter portions provide available banks or masses of metal which are reducible by suitable reduction techniques to a cross section equal to the desired ultimate cross section.

In the drawings:

FIGURE 1 is a flow sheet illustrating the several integral stages of operation in the production of the novel enlarged extruded shapes;

FIGS. 2 and 3 are transverse vertical sectional views of extruded shapes, shown in relation to the diameter circular die area, which shapes embody a single enlarged web or reservoir of metal in the rib portion of the shape;

FIG. 4 is a view similar to FIGS. 2 and 3, in which the rib portion of the extruded shape embodies a plurality of ribs or potentially reducible metal blanks;

FIG. 5 is a view similar to FIG. 3, in which the web portion of the extruded shape is of re-entrant or U configuration having a single rib;

FIG. 6 is a view similar to FIG. 5 in which a plurality of ribs is embodied in the web portion of the extruded shape;

FIG. 7 is a view similar to FIG. 2, showing ribs embodied in the vertical portions of the web; and

FIG. 8 is a schematic view illustrating the configuration of a typical design of an extruded shape, efficiently utilizing the circular die area, and showing the progressive and sequential or stage-wise reduction of the metal banks or ribs with accompanying lateral extension of the web.

As indicated hereinabove, the majority of metal extruder installations have a circular die diameter of 8 in. or less. With such extruders it is possible to obtain an extruded panel of somewhat greater width than the circular diameter of the die by first extruding a V-shaped configuration, and then flattening the shape into a panel of maximum width. In this manner, for example, a panel having a width of approximately 12 in. can be produced, using an 8 in. extruder, and a panel having a width up to 40 in. may be produced from a 24 in. extruder. It will be noted, however, that the preformed shape is merely flattened without any reduction in the cross-section of any portion of the shape. The novelty and profound economic significance of the invention can be readily assessed when it is considered that invoking its principles, in accordance with the present invention, permits the production of a shape of width up to 24 in. or more, using an extruder having a 5 in. diameter circular die area, and

70

shapes of a width up to 100 in. or more, when employing an extruder having a 24 in. diameter circular die.

The novel method of producing extruded shapes of enlarged dimensions will readily be understood from a consideration of the flow sheet of FIG. 1 in which the major producing units are shown diagrammatically. As there illustrated, the method essentially comprises extruding a shape of novel configuration or design in the extruder stage A, and subsequently subjecting such initially formed shape to progressive reduction of selected areas thereof in a series of reduction stages B, between units of which stages the particular shape may be thermally treated during the progress of reduction, and finally subjected to a suitable heat treatment in a heating zone C to improve its mechanical properties.

Considered more in detail, the extruder may be of any standard size of the type currently in use, comprising, essentially, a hydraulic cylinder 1, a ram 2, a die holder 3 and a runout table 4 attached to the die holder. Within the die holder there is mounted any one of the selected dies adapted to produce a shape of the cross sectional contour shown in FIGS. 2 to 6, inclusive. In operation, the cylinder-actuated ram forces an inserted homogenized, preheated ingot or billet through the die and the emergent shape 5 is received on the runout table; upon completion of the ram stroke, the table and die holder are advanced hydraulically, and the butt end of the ingot is cropped. The extruded shape may be allowed to cool, and may then be straightened by stretching beyond its yield strength to remove distortion and to equalize strains. The shape is then processed in the reduction stage B, during which operation the thickness of the ribs is progressively and sequentially reduced, and the metal embodied in a rib or ribs is displaced laterally of the longitudinal section of the shape, to thereby increase the width of the shape in proportion to the mass of metal incorporated in the rib portions of the as-extruded shape. In certain circumstances the described straightening operation may be omitted completely or it may be performed after completion of the rib reduction operation.

The rib reduction of the various extruded shapes may be progressively effected in any suitable manner; for example, by means of presses, power brakes, or other techniques, such as hot or cold roller reduction or combinations thereof. As shown in FIGS. 1 and 8, the metal reduction is effected in a series of tandem rolling machines comprised of any selected number of units 6, 7, 8 and 9. As will be appreciated, the number of such units employed or required will depend essentially on the cross sectional thickness of the rib or ribs, and on the number of individual ribs in a particular extruded shape. The roller reduction units may be of any suitable type, such as a two-high units shown, having rolls 10 and 11, mounted in the stand 12, and driven in the usual manner. As will be appreciated, the width and size of the rollers in the several units may vary, depending on the number of reduction passes required for any particular extruded shape, the width being selected to accommodate the increased width of the progressively laterally expanding extruded shape.

Interposed between certain of the roller stands, or between selected groups of tandem rolls, is one or more induction heating stages 13, 14 and 15, which may function as intermediate stress annealing stages during cold roll reduction, or as preheating stages during hot roll reduction, the temperatures of the stages being suitably controlled for these respective purposes, in accordance with current practice.

After final reduction of the ribs to the desired ultimate cross section, the shape may be heat treated in a horizontal or vertical heat-treat furnace 16, to modify its temper and improve the mechanical properties of wrought alloys amenable to heat treatment, and the shape then may be straightened in a suitable stretcher, not shown, to remove distortion and to relieve internal stresses. In

the case of wrought, non-heat treatable alloys, the temper may be strain hardened, strain hardened and partially annealed, or strain hardened and stabilized. With some of the shapes the final straightening may be effected on a roller straightener, not shown. The finished expanded shape thus produced may, if desired, be further treated by anodizing or the like, to improve its surface characteristics. Where greater accuracy and close tolerances are required, the shape may be pulled through a final sizing die. Similarly, if desired, the finished expanded extruded shape may be treated as by rolling or pressing to modify the contour or profile of any of the web or flange portions thereof.

In accordance with the present invention, the design and profile of the as-extruded shape is chosen to most effectively utilize the circular die area of the particular extruder, while insuring the incorporation of sufficient metal in the ribs or banks to provide for the subsequent lateral or vertical extension of selected sections of the shape during the roller reduction process. Any selected number of ribs may be embodied in the extruded shape, and the ribs may be of any desired configuration to most effectively correlate them with the particular reduction technique employed, and with the desired size and shape of the final product. Thus, the total mass of metal embodied in the rib portion which is to be reduced to the same cross section as the integral, initially formed web portion may be incorporated in a single rib or mass or may be divided or distributed between a plurality of smaller ribs or masses. The number of reduction passes or the number of pairs of rolls used in the reduction stage and, in the case of cold roll reduction, the number of intermediate anneals, will depend to a very considerable degree on the thickness of the ribs which are to be reduced; thus a thicker rib will require more reduction passes than one of thinner section. The number of passes will also depend, to some degree, on the configuration of the as-formed ribs, i.e., whether these are substantially circular, semi-circular, convex or the like, and also on the related configuration of the sections of the reducing rolls which contact the protuberant ribs. For a given shape the total mass of the to-be-reduced metal which is to be embodied therein, to secure any predetermined extension in one or more dimensions of the ultimate finished product, can readily be calculated and its distribution in the shape can be chosen to most effectively and economically insure its reduction.

The wide latitude of shape design permissible under the invention is illustrated in FIGS. 2 to 7, inclusive. These several designs, as will be appreciated, represent merely characteristic shapes and not the complete or exclusive range which may be utilized.

Referring to FIG. 2, there is shown a simple design of a shape producible according to the invention for the production, for example, of a panel structural member. This shape comprises a web member having a horizontal plate or web portion 17 and integral vertical legs 18 formed with terminal inturned flanges 19. Incorporated in the central portion of the plate or web 17, the total mass of metal which is to be subjected to reduction is in the form of a relatively elongated cylindrical section 20. The mass of metal in this rib or metal bank is that which has been previously calculated to give the desired lateral extension of the panel when such rib is progressively reduced by roller or power press reduction to the same cross section as the contiguous plate section 17. This shape represents the simplest form or design calculated to produce a desired extension with the minimum number of reduction passes and with minimum annealing.

In FIG. 3, there is shown a shape generally similar to that shown in FIG. 2, having the plate or web section 21, integral legs 22 with inturned flanges 23 and a metal bank or rib portion 24 in the form of a mass of circular cross section embodied in the central longitudinal portion of the web 21, the mass of which is sufficient to produce

a lateral extension of the panel equivalent to that formed from the shape shown in FIG. 2.

In FIG. 4 there is illustrated, in simple form, the subdivision of the total necessary metal bank into a plurality of reducible ribs. The shape comprises a web or plate section 25, integral vertical legs 26 formed with the in-turned flanges 27 and a metal bank comprising separate spaced ribs 28, 29 and 30 integrally embodied in the to-be-extended upper web or plate 25. Generally considered a shape of such design requires fewer reduction passes and fewer anneals than a shape of the type shown in FIG. 3. Such designed shape also simplifies the reduction process because the smaller ribs 28, 29, and 30 require less mechanical force to reduce them to the required web thickness and therefore can be reduced utilizing smaller, lighter and less expensive machinery, without limiting the ultimate size of the final finished product. This type of shape also insures more accurate control of the extension of the lateral dimension of the web to its desired ultimate width.

In FIG. 5 there is illustrated another form or design of an as-extruded shape in which the circular die area is utilized to initially form a greater portion of the ultimate width of the end product than the designs previously described. In such design the as-extruded shape comprises a relatively extensive web incorporating upper plate sections 31 having reentrant vertical extensions 32, of the same cross section as the contiguous sections 31, and integral vertical legs 33 terminating in terminal flanges 34. In this design a rib or metal bank 35 is embodied in the web between the extensions 32, such rib containing the mass of metal required to laterally elongate the upper web to the desired ultimate width. As will be appreciated, in processing this type of shape for the reduction of rib 35, the shape is first flattened to maximum width, the extensions 32 then constituting integral prolongations of the plate sections 31. Thereafter the rib 35 is reduced in the manner previously described.

In FIG. 6 there is shown an extruded shape design similar to that of FIG. 5, in which the calculated total mass of metal required for the desired extension of a web is distributed equally between a plurality of appropriately positioned ribs. The shape may comprise upper web portions 36 having integral reentrant extensions 37 and integral legs 38, each of which is formed with an in-turned flange 39. The as-extruded shape embodies rib sections 40 and 41 in the upper web portions 36, and a rib section 42 in the reentrant extension 37. As in the case of the shape shown in FIG. 5, prior to reducing the rib sections in the reduction rolls, the as-extruded shape is flattened by rolling or pressing to its maximum width wherein the web portions 36 and 37 constitute a continuous flat upper web.

As previously noted, the concept of embodying potentially reducible metal banks or ribs in an extruded shape to permit subsequent extenuation by reduction working of the metal may be invoked to widen preformed shapes of the type shown in FIGS. 2 to 6, or to deepen portions of the shape in FIG. 7. Referring to FIG. 7, the as-extruded shape comprises an upper flat web portion 43 of selected width and cross section, and integral angularly disposed legs 44 terminating in in-turned flanges 45. Embodied in the legs 44 are metal ribs 46 of a preselected mass which, when reduced to the same cross section as the legs, will extenuate the legs to the desired, preselected dimension. As will be understood, in the reduction stage the extruded shape is fed to the reduction rolls with the legs 44 in a horizontal position, parallel to the axes of the rolls. In this type of reduction the shape may be fed to a spaced, in-line series of roller stands comprised of a pair of tandem or two-high rolls vertically spaced a distance equal to the width of the web portion 43, and the ribs 46 in each leg may be reduced simultaneously and to the same degree or extent in each pass through the reduction units. More simply, if desired, the to-be-re-

duced shape may be fed to a series of typical longitudinally spaced tandem or two-high rolls to reduce the rib in one leg to a selected cross section, after which the shape may be inverted and repassed through such group of rolls to reduce the rib in the opposite leg to the same degree. The thus partially reduced shape may be then annealed, in the case of cold reduction, and the sequential, stage-wise reduction of the rib or ribs repeated to the extent necessary to secure the desired ultimate reduction. While the legs 44 are shown as having in-turned terminal flanges 45, these may be omitted in the as-extruded shape, and subsequently formed, by appropriate pressing or shaping operations, after the ribs have been completely reduced. As in the previous cases of extenuation of ribs in the upper web portion of a shape, the ribs embodied in the to-be-extruded leg portions of an extruded shape may be of any desired contour or profile best calculated and designed to achieve most efficient reduction by the particular design of the reduction rolls employed; thus the ribs may, as shown, be of circular cross section, however, for correlation with specially designed roller members the ribs may be of other profile or cross section, such as semicircular, ellipsoidal, semi-ellipsoidal, or the like.

The sequential phases of the direct line production of the novel expanded extruded shape will be seen from a consideration of FIGS. 1 and 8. In FIG. 8 there is shown a shape, extruded from a press having a circumscribed circle of 5 in. diameter, from which is ultimately produced a shape of panel configuration having a web width of 16 in. and a leg depth of 3.5 inches. It is to be particularly noted that the orthodox method of producing a shape of this width would require a press having a circumscribed circle of 18 in. diameter. The as-extruded shape comprises an upper web portion 47, integral leg portions 48 having the integral intermediate U-shape flange sections 49 and terminal U flanges 50. The upper web portion embodies a bank or mass of metal distributed in ribs 51, 52, 53, 54 and 55, which are equally spaced apart and are of equal cross section. In this illustrative shape the cross section or wall thickness of the web and leg portions is 0.0625 in., and the area of each of the integral ribs is 0.1936 inches. When these several ribs are reduced to the same cross section as that of web 47 the area of the panel in the upper web is increased by 0.78125 sq. in. per foot of the panel section.

As will be seen in FIG. 1, as the shape is extruded it is received on the runout table 4 and the butt end is sheared or cropped, and while still hot it is fed to the direct line of the metal reduction units and passed sequentially through the units. In such direct or immediate passage of the extruded shape to the roller mills its temperature (extrusion temperature) is of the order of 380° to 420° C., and hence it is thermally prepared for hot rolling operations; however, if desired, the shape may be additionally heated, as by induction heating, to raise the temperature to some higher optimum. Since the as-extruded shape is of fine grained structure and is precision formed, no scalping is required prior to hot roll reduction.

In the process of reducing the metal ribs, and commensurately extending their mass into a continuous web of selected thickness, the ribs are reduced in stages; thus, as is illustrated in FIG. 8, in extending the upper web the central rib 53 is first reduced to a selected cross section in one stage, and thereafter the ribs 52 and 54 are simultaneously reduced in a second stage, and then the ribs 51 and 55 are reduced in the final stage so that the web is progressively laterally extended from the center of the web section outwardly towards the sides of the panel. In the preferred operation, the metal reduction of the ribs may be effected in three phases, namely, a primary break down or hot rolling operation in which, in a series of passes a rib is reduced by from approximately 60 to 90 percent of the desired ultimate reduction, while maintaining its

crystalline structure; an intermediate roughing cold rolling, to effect a reduction in thickness, close to the ultimate desired reduction, and a finishing or planitizing rolling operation, between smooth highly finished rolls, with but slight reduction to give a hard surface and to establish accurate, uniform thickness of the web within narrow limits. In the preliminary roughing or hot rolling phase of the rib reduction, it is advantageous to use small diameter rolls because of their deeper bite or nip into the metal, and larger diameter rolls for the intermediate and finishing reductions. When small diameter rolls are used it is desirable to employ three-high or four-high stands to insure the rigidity of the rolls.

The stage-wise reduction of the ribs and the consequent progressive lateral extension of the upper web is depicted in FIG. 8. As there shown, the rib 53 which may be at a temperature of 380° C. to 420° C. or more, is worked in a selected number of passes until it is reduced in cross section passing from its original circular form to assume a generally flattened and widened section shown at 56 to 58. Such reduction may be effected by employing a series of in-line roller stands or, if desired, in a reversing mill. At such stage of reduction the temperature of the shape is lowered to a point where further reduction (cold rolling) results in some work hardening, and at this stage the shape may be reheated, utilizing an induction or the furnace heater 13, and additional hot rolling continued, or the partially reduced rib 56 may be further reduced in a selected number of cold roll passes until it assumes a wider and thinner form as shown at 58. At this point, if the reduced metal section is work hardened to an undesired extent the piece may be rapidly annealed in one of the furnaces shown in FIG. 1 and then subjected to further reduction in an in-line series of roller mills, or in a single reversing mill, until the reduced segment or section 58 is of the same cross section as, and co-extensive with, the web portion between the unreduced ribs 52 and 54.

In the next stage of reduction, as previously explained, the ribs at the termini of the reduced section 58 are simultaneously and progressively reduced in a series of similar stage-wise reductions, such ribs being progressively reduced or flattened to form sections 59, 60, and 61.

In the third stage a similar series of roller reductions is carried out to reduce the ribs 51 and 55 to the progressively reduced sections 62, 63, and 64. The shape may then be straightened, if required, by stretching or by roller straightening to produce the final shape in which the legs 48 are identical in shape and dimensions as in the as-extruded shape, whereas the original web portion embodying the several ribs comprises a continuous widened web of uniform cross section. When the shape produced is comprised of a heat treatable wrought alloy it may be of any selected temper, either as fabricated or annealed, or it may be given any desired higher temper, such as T<sub>3</sub>, T<sub>4</sub>, T<sub>5</sub>, T<sub>6</sub> or T<sub>8</sub> by suitable treatment in a thermal treating stage 16. When the shape is comprised of a non-heat treatable alloy the temper may be, as fabricated, strain hardened only, strain hardened and then stabilized, etc.

It will be understood that the rollers in the several roller mills employed in the different stages of rib reduction are correlated in size and design with the profile of the shape processed therein, so that the rollers selectively contact only the rib or ribs undergoing reduction in the different stages; thus the rollers mounted in the stands used in the reduction of rib 53 are so designed as to contact and reduce such rib without any reductive action on adjacent ribs 52 and 54; similarly, the rollers mounted in the stands used in the reduction of ribs 52 and 54 are designed to contact and progressively reduce these two ribs without affecting the contour of adjacent ribs 51 and 55. For this purpose the rollers may be of a shape or profile specially designed for its particular operation, for example, the rollers may be of a generally cylindrical form having a section or sections of modified diameter or camber so

positioned along the axis of the rolls as to contact only the rib or ribs which are to be reduced. As is known in the usual type of rolling operations, the rolled metal has a plane of symmetry and the reduction of the metal tends to elongate it in a plane of symmetry normal to the axes of the rolls with but little spread being produced in its width; in such typical rolling operations the piece or slab subjected to rolling contact can elongate because there are no restrictive forces opposing such elongation. In the rolling operations described herein the normal tendency of the ribs of the web to elongate is opposed or restricted by their integral lateral web extensions which are not being worked or reduced, and hence the tendency of the rib to elongate is opposed by the adjoining tensioned, diametrically positioned web sections. The lateral component of movement of the metal undergoing reduction is less restricted, such restriction being imposed only by the inherent stiffness of the relatively thin web section whose side edges are unconfined, thus allowing the web to be displaced laterally. It will be appreciated that the lateral component of the force tending to widen the upper web portion can be increased by proper design of the camber of the rib-contacting portions of the rolls.

The extended extruded shapes, produced according to the present invention, may be given a surface finish best adapted to improve their appearance, usefulness and endurance for any general or special intended use; thus the shapes may be given any of the mechanical, chemical or electrochemical finishes to which aluminum alloys are amenable. The individual unit shapes produced as described herein may be joined by any applicable welding technique to produce a great variety of larger integral forms and shapes for use in various fields of construction.

While I have shown and described the preferred embodiment of my invention, I wish it to be understood that I do not confine myself to the precise details set forth by way of illustration, as it is apparent that many changes and variations may be made therein, by those skilled in the art, without departing from the spirit of the invention or exceeding the scope of the appended claims.

I claim:

1. A process of producing an extruded metallic shape of a width substantially greater than the diameter of the circumscribed circle of the die orifice of an extrusion press, comprising extruding a shape having a web portion of uniform cross-section and an integral mass of substantially greater cross-section than the cross-section of the web portion, said mass providing a material bank of formable metal, subsequently passing the extruded shape through a series of reduction zones and progressively reducing the cross-section of the material bank to progressively extend the width of the shape while maintaining the cross-section of the web portion until the cross-section of the material bank is equal to that of the web portion.

2. A process, in accordance with claim 1, in which the extruded shape is comprised of a ferrous metal.

3. A process in accordance with claim 1, in which the extruded shape is comprised of a non-ferrous metal.

4. A process according to claim 1, in which the extruded shape is comprised of a non-ferrous alloy.

5. A process according to claim 1, in which the extruded shape is comprised of a ferrous alloy.

6. A process in accordance with claim 4, in which the non-ferrous alloy is chosen from the group consisting of aluminum and magnesium base alloys.

7. A process of producing an extruded shape of a metallic alloy of a width substantially greater than the diameter of the circumscribed circle of the die orifice of an extrusion press, comprising extruding a shape having a web portion of uniform cross-section and of parallel integral, longitudinal ribs of substantially greater cross-section than the cross-section of the web portion, subsequently passing the extruded shape through a series of reduction zones and progressively reducing the cross-section of the ribs while progressively extending the width

of the shape until the cross-section of the rib is equal to that of the web portion.

8. A process according to claim 7, in which hot reduction is effected in said reduction zones.

9. A process according to claim 7, in which hot rolled reduction is effected in said reduction zones.

10. A process according to claim 7, in which cold reduction is effected in said reduction zones.

11. A process according to claim 7, in which cold rolled reduction is effected in said reduction zones.

12. A process according to claim 7, in which the mass of metal embodied in the integral longitudinal rib exceeds that embodied in the web portion.

13. A process of producing extruded, wide web shapes of metallic alloys which comprises extruding a shape having web portions of uniform cross-section of the desired ultimate thickness and integral portions of substantially greater thickness than the said web portions extending lengthwise of the extruded shape; continuously passing the extruded shape through a series of reduction zones and therein selectively and progressively reducing the cross-sections of said integral portions while progressively extending the width of the shape until the cross-sections of the integral portions equal that of the web portions.

14. A process, according to claim 13, in which hot reduction is effected in said reduction zones.

15. A process, according to claim 13, in which cold reduction is effected in said reduction zones.

16. A process, according to claim 13, in which hot reduction is effected in certain of said reduction zones and cold reduction is effected in the other reduction zones.

17. A process, according to claim 13, in which the said shape is annealed between selected zones of the series.

18. A process, in accordance with claim 13, in which the shape is subjected to inductive heating prior to passage through certain of the series of reduction zones.

19. A process, according to claim 13, in which the mass of metal embodied in the said integral portions exceeds that embodied in the web portions.

20. A process, according to claim 13, in which the width of the shape after final reduction is at least twice that of the initially extruded shape.

21. A process, according to claim 13, in which the metallic alloy is a non-ferrous alloy.

22. A process for producing extruded shapes of a non-ferrous alloy of a width considerably greater than the limiting width of light press extruders having a circumscribed circle die orifice of the order of 5 to 8 inches, which comprises initially extruding a shape from such alloy, said extrusion embodying web portions of selected ultimate thickness and a thicker intermediate portion extending the full length of the shape, said intermediate portion embodying a mass of metal considerably greater than that of the web portions; progressively passing the extruded shape through a series of reduction zones and progressively reducing the cross-section of the said thicker intermediate portion while progressively extending the width of the shape until the cross-section of the intermediate portion equals that of the initially formed webs.

References Cited in the file of this patent

UNITED STATES PATENTS

|              |                 |               |
|--------------|-----------------|---------------|
| 1,040,614    | Bradley         | Oct. 8, 1912  |
| 2,023,827    | Wallmann et al. | Dec. 10, 1935 |
| 2,437,127    | Richardson      | Mar. 2, 1948  |
| 30 2,533,227 | Delaney         | Dec. 12, 1950 |
| 2,617,179    | Burke           | Nov. 11, 1952 |
| 2,692,421    | Cozzo           | Oct. 26, 1954 |
| 2,716,805    | Reed            | Sept. 6, 1955 |
| 35 2,741,834 | Reed            | Apr. 17, 1956 |
| 2,827,944    | Grossu          | Mar. 25, 1958 |